

Patented Sept. 11, 1923.

1,467,493

## UNITED STATES PATENT OFFICE.

CHARLES WILFRED PALMER AND WILLIAM ALEXANDER DICKIE, OF SPONDON, NEAR DERBY, ENGLAND, ASSIGNEES TO HENRY DREYFUS, OF LONDON, ENGLAND.

### MANUFACTURE OF ARTIFICIAL FILAMENTS, THREADS, AND FILMS.

No Drawing.

Application filed December 20, 1921. Serial No. 523,759.

*To all whom it may concern:*

Be it known that we, CHARLES WILFRED PALMER and WILLIAM ALEXANDER DICKIE, subjects of the King of Great Britain, both 5 of Spondon, near Derby, England, have invented certain new and useful Improvements Relating to the Manufacture of Artificial Filaments, Threads, and Films, of which the following is a specification.

10 It has been proposed to manufacture artificial filaments and films from solutions of cellulose acetate in organic solvents that are soluble in or miscible with water, by squirting or extruding the cellulose acetate solutions into aqueous coagulating baths.

Hitherto it has not been possible to obtain strong and elastic filaments or films by such methods owing to the fact that the cellulose acetate is not coagulated by water 20 in the form of a structurally continuous gel, but with a discontinuous granular or reticulated internal structure, so that the resulting threads or films are lacking in strength and elasticity.

25 In the specification of another application for patent Serial No. 523,758, filed December 19, 1921 we have proposed, with a view of obviating this difficulty to add ammonium thiocyanate or other thiocyanates to the coagulating baths, it having been found that 30 said thiocyanates are capable, owing to a latent solvent power which they have for cellulose acetate, of exerting a swelling and coagulation controlling action on the coagulating filaments or films and thereby tending 35 to preserve continuity of structure and to prevent the too complete shrinkage of the cellulose acetate which ordinarily occurs as the result of the removal of the organic solvent by the aqueous coagulating bath and causes precipitation of the cellulose acetate 40 with a discontinuous structure.

According to the present invention we employ in the aqueous coagulating bath, 45 solvents or latent solvents of cellulose acetate which are soluble in or otherwise miscible with water. We have found that such substances have a swelling and coagulation controlling effect on the cellulose acetate extruded into aqueous coagulating baths containing them. Such solvents or latent solvents are hereinafter referred to as swelling 50 and coagulation controlling agents.

As examples of such swelling and coagulation controlling agents may be mentioned,

acetone, diacetone alcohol, acetic acid, or formic acid, or mixtures of any of these, also aqueous solutions of zinc chloride or other salts which like the thiocyanates have a latent solvent power for cellulose acetate. 60

According to the present invention we add the swelling and coagulation controlling agents to the coagulation baths.

The invention applies in particular to the manufacture of artificial filaments, 65 threads, or films from acetone-soluble cellulose acetates, but may also be employed with other acetates of cellulose.

The solvents or latent solvents employed as swelling and controlling agents according to the invention must be used in sufficient quantity or concentration to exert the required modifying influence on the shrinking action of the water, but not in such quantity or concentration as to exert too great a 70 solvent power and prevent coagulation of the cellulose acetate.

In carrying out the invention, solutions of cellulose acetate in any organic solvents miscible with water or soluble in water may 80 be employed, for example acetone, or acetone-alcohol mixtures.

In carrying out the invention we may work for instance as follows, it being understood that this example is given by way of 85 illustration only and is in no way limitative.

A 16 per cent solution of cellulose acetate in acetone is forced in the known way through the capillary orifices of spinning nozzles into an aqueous bath containing a suitable quantity of acetone, diacetone alcohol, alcohol, or other solvent or latent solvent for example about 10-50 parts of acetone, or about 100 parts of alcohol, or about 5 parts of diacetone alcohol or acetic acid, per 100 parts of 90 water.

The coagulated filaments are carried through the bath under a guide and are wound up continuously in any known way. The swelling agent carried forward in the 100 thread is removed by washing, and the purified threads of cellulose acetate are dried.

The filaments issuing from the squirting nozzle are endowed with considerable strength and the combined action of the 105 water and swelling agent are such that the cellulose acetate solutions may be drawn out to filaments of great tenuity from orifices of relatively large diameter. In this way it is possible to obtain artificial silk filaments of 110

very low denier, for example as fine as 1 or 2 denier, i. e. as fine as natural silk.

It is understood that the limits of concentration of the swelling and coagulation 5 controlling agent may be varied to suit desired conditions.

What we claim and desire to secure by Letters Patent is:—

1. In a process for the manufacture of 10 filaments, threads or films, extruding cellulose acetate in solution into an aqueous coagulating bath containing an agent capable of swelling and controlling coagulation of the cellulose acetate, said agent being miscible with water.
2. In a process for the manufacture of 15 filaments, threads or films, extruding a solution

comprising cellulose acetate and an organic solvent thereof miscible with water, into an aqueous coagulating bath containing an 20 agent capable of swelling and controlling coagulation of the cellulose acetate, said agent being miscible with water.

3. In a process for the manufacture of filaments, threads or films, extruding a solution 25 of cellulose acetate in acetone into an aqueous coagulating bath containing acetone.

In testimony whereof we have hereunto subscribed our names.

CHARLES WILFRED PALMER.  
WILLIAM ALEXANDER DICKIE.

Witnesses:

THOS. H. COOK,  
A. A. GUNNING.